

1

2,934,583

## ANODE FOR MAGNESIUM PRIMARY CELLS

John A. Stevens, Midland, Mich., assignor to The Dow Chemical Company, Midland, Mich., a corporation of Delaware

No Drawing. Application February 13, 1958  
Serial No. 714,964

6 Claims. (Cl. 136—100)

This invention relates to an improved anode for use in a primary magnesium battery cell whereby the normal delayed action usually resulting from the employment of such a battery cell is decreased.

It has been well established that primary cells utilizing magnesium as the anode, manganese dioxide mixed with carbon as the cathode, and a bromide of an alkali metal, alkaline-earth metal, or ammonium as the electrolyte have specific advantages in certain uses. For example, a greater capacity per unit of volume is generally achieved with less weight. One of the primary disadvantages in utilizing magnesium as an anode for a primary cell is that the cells do not always attain full working voltage immediately on attempting to reuse them following a rest period. This delayed action may vary from 0 to as much as 100 seconds or more depending upon the specific composition of the components of the cell, the amount of use that has been made of the cell, the intervening resting period, and the age of the cell.

It is a principal object of the present invention to provide an anode material which results in a shorter delayed action when employed in the conventional magnesium primary cell. Still another object of the present invention is to provide such an anode material which comprises a conventional magnesium anode having small amounts of indium alloyed therein. Another object of the present invention is to provide such a magnesium anode material for primary cells containing from 0.03 to 1.7 percent indium alloyed therein. Other objects will become apparent hereinafter.

The foregoing and additional objects have been accomplished by providing a magnesium cell containing a magnesium anode, said magnesium anode containing from 0.03 to 1.7 percent indium alloyed therein.

Magnesium batteries have been described in a number of U.S. patents, including Nos. 2,547,907, 2,616,940, 2,712,564, etc. These patents all rely on a magnesium anode, a cathode into which has been mixed a depolarizing agent such as manganese dioxide, an alkaline metal,

2

alkaline-earth metal, or ammonium bromide electrolyte, an anode liner and a carbon current collector. The present invention specifically relates to an improvement in the anode of such a cell whereby the delayed action is substantially reduced. Provision of such an anode is accomplished by providing a magnesium alloy containing from 0.03 to 1.7 percent indium, preferably from 0.1 to 0.2 percent indium. The indium is added in conventional alloying techniques to the alloy melt and in 5 a conventional manner, the resulting material settled, poured, pickled, extruded, rolled, or cast to form the desired style and shape of anode. Various of the well-known magnesium anodes are improved by the addition of indium thereto. Representative alloy materials which 10 are suitable are those magnesium-base alloys containing at least 80 percent, and preferably 90 percent magnesium, containing from 1 to 12 percent aluminum, from 0.0 to 3.0 percent zinc, from 0.0 to 0.5 percent calcium, the balance being commercial magnesium containing not 15 over 0.005 percent iron, not over 0.002 percent nickel, and not over 0.6 percent manganese.

The anodes so provided are used in a conventional manner in a magnesium primary cell. The advantages of employing such an alloy are many, but primarily are 20 25 represented in the decreased delayed action of the cell.

The following examples are given to illustrate the anodes of the present invention, but are not to be construed as limiting the invention thereto:

30

### Example 1

Two alloy compositions, one of which contains 3 percent aluminum and 1.0 percent zinc, and 0.2 percent calcium, the remainder being commercial magnesium 35 (AZ31A), the second of which contains 3 percent aluminum, 1.0 percent zinc, the remainder being magnesium (AZ31B) were both treated so as to provide varying quantities of indium alloyed therein. Cells containing these alloys as anodes, a cathode of 91 percent manganese 40 dioxide, 3 percent barium chromate and 6 percent acetylene black, and an electrolyte containing 250 grams per liter of magnesium bromide and 0.36 gram per liter of sodium chromate were employed. Different cells containing the anodes of the present invention and comparison anodes were tested in 2 standard tests: the "Railroad Lantern" test utilizing an alternate discharge time and a rest time of 30 minutes during an 8-hour day with a subsequent rest time of 16 hours, 7 days per week, on a 32 ohm load for a three cell pack; and, the "General Purpose" test of 5 minutes per day discharge through 4 ohms per cell, 7 days per week.

50 The following table summarizes the results obtained from these tests:

| Base Alloy | Percent<br>In | Fabricated<br>State * | Delay in Seconds,<br>Railroad Lantern |      |      |      | General<br>Purpose |       | Anode<br>Eff.<br>General<br>Purpose |  |
|------------|---------------|-----------------------|---------------------------------------|------|------|------|--------------------|-------|-------------------------------------|--|
|            |               |                       | A.M.                                  |      | P.M. |      | Max.               | Ave.  |                                     |  |
|            |               |                       | Max.                                  | Ave. | Max. | Ave. |                    |       |                                     |  |
| AZ31A      | 0             | 4                     | 5.5                                   | 4.8  | 15   | 11.3 | -----              | 1.5   | 55.4                                |  |
| AZ31A      | .05           | 3                     | 6.0                                   | 4.7  | 2    | 1.2  | 6                  | 2.3   | 55                                  |  |
| AZ31A      | .15           | 1                     | 6.0                                   | 3.2  | 1    | 0.1  | 3                  | 2.4   | 54                                  |  |
| AZ31A      | .15           | 2                     | 6.0                                   | 3.9  | 2    | 0.6  | 3                  | 2.2   | 54                                  |  |
| AZ31B      | 0             | 2                     | 30                                    | 21   | 42   | 20   | 3                  | 1.5   | 53                                  |  |
| AZ31B      | .02           | 3                     | 29                                    | 21   | 2    | 1.6  | 2.0                | 1.4   | 54                                  |  |
| AZ31B      | .05           | 2                     | 32                                    | 21   | 7    | 2.3  | 2.0                | 1.2   | 53                                  |  |
| AZ31B      | .12           | 3                     | 16                                    | 12   | 2    | 0.1  | 4.0                | 1.6   | 53                                  |  |
| AZ31B      | .51           | 3                     | 18                                    | 10   | 0    | 0    | 2                  | 0.9   | 46                                  |  |
| AZ31B      | 1.38          | 4                     | 16                                    | 1.8  | 0    | 0    | -----              | ----- | -----                               |  |

\* (1) As-rolled. (2) As-rolled, annealed 300 C. for  $\frac{1}{2}$  hour. (3) As-rolled, annealed 700 C. for  $\frac{1}{2}$  hour. (4) Impact extruded battery cans.

## Example 2

A series of D-sized cells having standard steel jacket construction were employed in the following tests. In Group No. 1, the anode was a .025 inch sheet containing 3.5 percent aluminum, 0.24 percent calcium, 0.96 percent zinc, and 0.13 percent indium, the balance being magnesium. The cells from Group 2 containing a similar sheet anode alloyed from 3.1 percent aluminum, 0.17 percent calcium, 0.86 percent zinc, 0 percent indium. These anodes were employed with an electrolyte consisting of 400 grams per liter of magnesium bromide, and 0.36 gram per liter of sodium chromate solution. The cathode mix was 87 percent manganese dioxide, 3 percent barium chromate, 10 percent acetylene black and 0.25 percent magnesium powder. It was wet with 440 milliliters of electrolyte per thousand grams of dry material. The weight of the wet cathode mix was 54 grams per cell. These cells were hooked five in a series to make a nine volt pack. Each nine volt pack was employed in an R.C.A. Transistor Radio 7-B-10K maintained at a predetermined volume of nine milliamperes and the delay measured by determining the time required to reach this volume. The series of cells were discharged 2 hours per day through 900 ohms to an end voltage of 6 volts. The delay average was determined over this period and the delay was measured at the beginning of the two hour discharge. This test resulted in the following results:

|               | Max. | Ave. |
|---------------|------|------|
| Group I.....  | 2.3  | 0.1  |
| Group II..... | 15.0 | 9.5  |

35

Various modifications may be made in the present invention without departing from the spirit or scope thereof and it is to be understood that I limit myself only as defined in the appended claims.

I claim:

1. A magnesium battery anode comprising principally

4  
magnesium having 0.03 to 1.7 percent indium alloyed therein.

2. A magnesium battery anode comprising: from 1 to 12 percent aluminum, 0.0 to 3.0 percent zinc, 0.0 to 0.5 percent calcium, 0.03 to 1.7 percent indium, balance magnesium.

3. A magnesium battery anode comprising: from 1 to 12 percent aluminum, 0.0 to 3.0 percent zinc, 0.0 to 0.5 percent calcium, 0.03 to 1.7 percent indium, less than 0.005 percent iron, less than 0.002 percent nickel, less than 0.6 percent manganese, the balance being magnesium.

4. In a magnesium battery which includes a cathode of manganese dioxide mixed with a carbon, a magnesium anode, a bromide electrolyte, and a carbon current collector, the improvement which comprises: providing said magnesium anode having 0.03 to 1.7 percent indium alloyed therein.

5. In a magnesium battery which includes a cathode of manganese dioxide mixed with carbon, a magnesium anode, a bromide electrolyte, and a carbon current collector, the improvement which comprises: providing an anode which includes from 1 to 12 percent aluminum, 0.0 to 3.0 percent zinc, 0.0 to 0.5 percent calcium, 0.03 to 1.7 percent indium, the balance being magnesium.

6. In a magnesium battery which includes a cathode of manganese dioxide mixed with carbon, a magnesium anode, a bromide electrolyte, and a carbon current collector, the improvement which comprises: providing an anode which includes: from 1 to 12 percent aluminum, 0.0 to 3.0 percent zinc, 0.0 to 0.5 percent calcium, 0.03 to 1.7 percent indium, less than 0.005 percent iron, less than 0.002 percent nickel, less than 0.6 percent manganese, the balance being magnesium.

## References Cited in the file of this patent

## UNITED STATES PATENTS

2,683,184 Boswell \_\_\_\_\_ July 6, 1954  
2,836,645 Morehouse et al. \_\_\_\_\_ May 27, 1958

## FOREIGN PATENTS

1,081,155 France \_\_\_\_\_ June 9, 1954

40